# EUROPEAN PATENT SPECIFICATION

(11) **EP 3 704 286 B1**
(45) Date of publication and mention of the grant of the patent: **06.12.2023**
(21) Application number: 18804756.7
(22) Date of filing: 25.10.2018
(51) Int. Cl.: C23C 22/10, C23C 22/08, C23C 22/33

(54) **PROCESS AND COMPOSITION FOR TREATING METAL SURFACES USING TRIVALENT CHROMIUM COMPOUNDS**
VERFAHREN UND ZUSAMMENSETZUNG ZUR BEHANDLUNG VON METALLOBERFLÄCHEN UNTER VERWENDUNG DREIWERTIGER CHROMVERBINDUNGEN
PROCÉDÉ ET COMPOSITION POUR TRAITER DES SURFACES MÉTALLIQUES À L'AIDE DE COMPOSÉS DE CHROME TRIVALENT

(30) Priority: 30.10.2017 US 201762578787 P
(43) Date of publication of application: 09.09.2020
(73) Proprietor: BULK CHEMICALS, INC., Reading, PA 19605 (US)
(72) Inventor: RIVERA, Jose, B., Auburn PA 17922 (US); HANNA, Cody, Lancaster PA 19602 (US)
(74) Representative: Cantaluppi, Stefano
(86) International application number: PCT/US2018/057533
(87) International publication number: WO 2019/089347

(56) References cited:
- EP-A1- 0 532 779
- EP-A1- 1 484 432
- EP-A1- 1 712 524
- EP-A1- 2 060 660
- GB-A- 2 201 157
- JP-A- S4 935 432
- JP-A- H01 123 081

## Description

### TECHNICAL FIELD

This invention relates generally to compositions and the use of such compositions for passivating and improving the paint adhesion of metal surfaces. The composition may be used as a pre-paint treatment and is intended to be used to treat a range of metals including copper, brass, magnesium, aluminum, iron, zinc, cadmium, or alloys thereof. More particularly, this invention relates to an aqueous composition, suitable for use as a dried-in-place coating for metal, that comprises trivalent chromium, phosphate, silica, and hydrogen peroxide and methods for using that composition. The process and seal coat have been found to demonstrate good paint adhesion results.

### BACKGROUND OF THE INVENTION

Known methods of treating metal surfaces to improve paint adhesion and corrosion resistance of painted metal surfaces include two general classes of chemistries. The first class is based on traditional conversion coating types of chemistries, such as zinc phosphate, iron phosphate, chromium chromate, chromium phosphate, etc. The second class is based on more recent developments in the metal pretreatment industry and is characterized by what is now referred to as "dried-in-place" technology. Traditional conversion coating chemistries require rinsing of the metal substrate to remove applied pretreatment solution. Dried-in-place chemistries allow for the applied solutions to be dried on the metal substrate to which they are applied, without rinsing prior to the application of a paint.

With regard to dried-in-place processes, it is generally known to treat the surfaces of metals, such as iron, zinc, cadmium, aluminum, or alloys thereof with aqueous hexavalent chromium solutions which contain chemicals that dissolve the surface of the metal and form insoluble films known as "chromate conversion coatings." These coatings, which contain hexavalent chromium, are corrosion resistant and protect the metal from various elements which cause corrosion. In addition, it is known that hexavalent chromate conversion coatings generally have good paint bonding characteristics and, therefore, provide an excellent base for paint or other finishes.

Although the aforementioned coatings enhance corrosion resistance and paint bonding properties, the coatings have a serious drawback. Hexavalent chromium shows toxicological effects and has been determined by the Environmental Protection Agency as a risk to the environment and by the Occupational Safety and Health Agency as a health risk. Moreover, chemistries based on hexavalent chromium are classified as carcinogens by these agencies.

Within the past few decades, various compositions and processes, not relying on hexavalent chromium, have been described and used for treating metal surfaces. One such example is described in U.S. Pat. No. 4,169,741 to Rausch et al., which describes a dried-in-place method using a composition comprising, among other elements, trivalent chromium, phosphate ion, and dispersed silica. Examples of aqueous compositions for treating metal surfaces comprising silica and Cr(H₂PO₄)₃ are disclosed in GB2201157 A, JP 54935432 A, EP 2060660 A1, EP 0532779 A1, JP H01123081 A EP 1484432 A, and EP 1712524 A1.

It is highly desirable to provide coatings and processes which are free of hexavalent chromium, but still capable of improving paint adhesion and corrosion resistance of metal surfaces, such as aluminum, which are comparable to conventional hexavalent chromium-based coatings. Additionally, there is a need to provide protective coatings having excellent corrosion resistance with lowered resistivities and adequate coating weights.

### BRIEF SUMMARY OF THE INVENTION

The present invention relates to a composition for treating a metal surface to improve paint adhesion and corrosion resistance and/or maintain low electrical contact resistance. In an aspect of the present invention, there is provided a composition consisting of water, a trivalent chromium compound with the formula Cr(HₓPO₄)₃, where x is 2, a silica compound, and optionally hydrogen peroxide.

In another aspect of the present invention, there is provided a composition consisting of water, a trivalent chromium compound with the formula Cr(HₓPO4)₂ where x is 1.5, a silica compound, and optionally hydrogen peroxide.

In an embodiment, the trivalent chromium compound is present in an amount of between: about 10% wt. % to about 5% wt. %; about 10% wt. % to about 2.5% wt. %, about 10% wt. % to about 1% wt. %, or about 10% wt. % to about 0.5% wt. %..

In another embodiment of the invention, the silica is present in an amount of less than 2% wt. %; less than 1.75% wt. %; or less than 1.5% wt. %.

In still another a aspect of the present invention, there is provided a process for treating a metal surface. The process includes the step of contacting the metal surface with a composition of claims 1 or 5.

In an embodiment, the process for treating a metal surface comprises the steps of: (1) cleaning the metal surface to form a cleaned metal surface; (2) rinsing the cleaned metal surface with water to form a rinsed metal surface; and (3) contacting the rinsed metal surface with a composition of claims 1 or 5.

In a still further embodiment, the process additionally comprises, after contacting the rinsed metal surface with the composition, again rinsing the metal surface with water and then sealing the metal surface.

The processes may additionally comprise, before the first contacting step, the step of cleaning the metal surface with an alkaline cleaner and rinsing. The processes may further comprise, after contacting the metal surface with the pretreatment composition, the steps of rinsing the metal surface with water and then painting the surface of the metal. The pH of the aqueous pretreatment composition is preferably acidic and more preferably has a pH of between about 1 and about 4.

It is to be understood that both the foregoing general description and the following detailed description are exemplary, but are not restrictive, of the invention.

### BRIEF DESCRIPTION OF THE DRAWING

The invention is best understood from the following detailed description when read in conjunction with the accompanying drawing. It is emphasized that, according to common practice, the various features of the drawing are not to scale. On the contrary, the various features are arbitrarily expanded or reduced for clarity. Included in the drawing are the following figures:
FIG. 1 is a side-by-side photograhic comparison of the results from Composition 1 as compared to the Control composition for panels scribed and exposed to neutral salt spray for a period of 250 hours per ASTM B117;
FIG. 2 is a side-by-side photographic comparison of the results from Composition 1 as compared to the Control composition for panels scribed and exposed to neutral salt spray for a period of 250 hours per ASTM B117;
FIG. 3 is a side-by-side photographic comparison of the results from Composition 1 and Composition 2 as compared to the Control composition for panels scribed and exposed to neutral salt spray for a period of 500 hours per ASTM B117;
FIG. 4 is a side-by-side photograph of the results from Composition 2 for panels scribed and exposed to neutral salt spray for a period of 250 hours per ASTM B117;
FIG. 5 is a side-by-side photographic comparison of the results from Composition 1 as compared to the Example 1 composition disclosed in the Rausch patent for panels scribed and exposed to neutral salt spray for a period of 250 hours per ASTM B117; and
FIG. 6 is a side-by-side photographic comparison of the results from Composition 1 as compared to the Example 1 composition disclosed in the Rausch patent for panels scribed and exposed to neutral salt spray for a period of 250 hours per ASTM B117.

### DESCRIPTION OF THE INVENTION

The present invention is directed to compositions and processes for treating a metal surface. Compositions according to the present invention consist of water, a trivalent chromium compound with the formula Cr(HₓPO₄)₃, where x is 2, or with the formula Cr(HₓPO₄)₂, where x is 1.5, a silica compound, and optionally hydrogen peroxide. Processes according to the present invention include contacting a metal surface with the above compositions.

Aqueous compositions of the present invention are applied to a metal surface after cleaning but before some final coat is applied to the metal surface, contributing to at least one of the following: (1) improving the paint adhesion of the metal surface; (2) improving the corrosion resistance of the metal surface; and (3) maintaining or reducing the resistivity of the metal surface. Compositions of the present invention include compositions which significantly improve one or two of these characteristics, even though at least one of the others is worsened to a lesser extent. The improvement could be due to the compositions alone or the compositions in combination other process steps. Such compositions are referred to herein or in the metal treatment industry as pretreatment compositions, conversion coatings, or working compositions. "Resistivity" is defined as resistance per unit surface area.

As used herein, the term "hexavalent chromium compound" means compounds, namely salts, of chromium in which the chromium has a valence of plus 6. A wide range of anions could be used, and more than one hexavalent chromium compound could be used. Preferably, the hexavalent chromium compound is anhydrous chromic acid (CrO₃), chromic acid (H₂CrO₄), or chromium chromate (Cr₅O₁₂).

As used herein, the term "metal," used for example in the phrase "metal surface," includes copper, brass, magnesium, aluminum, iron, zinc, cadmium, or alloys thereof. Each metal listed includes both the elemental metal and alloys thereof; for example, the term "aluminum" means aluminum and aluminum alloys. The term "alloy" is a metal in which the primary element has a higher content than every other element or a content equal to the highest content of every other element (e.g., an aluminum alloy being a metal in which aluminum is present in an amount at least equal to that of any other element). Iron alloys include cold rolled steel, electro-galvanized steel, and hot-dipped galvanized steel. Preferably, compositions of the present invention are used to treat a range of metals including alloys of copper, brass, magnesium, aluminum, and iron.

As used herein, the term "pretreatment composition" means any composition which improves the paint adhesion and corrosion resistance of a metal surface. Aqueous pretreatment compositions are used as a pretreatment before painting and may be used as a passivation treatment to reduce the formation of corrosion in the uncoated (unpainted) condition. Thus, although the composition may be called a pretreatment composition for convenience, it is a composition used for pretreatment (i.e., improving the adhesion of subsequently applied paint) and passivation (i.e., resisting corrosion of the unpainted surface).

As used herein, the term "treating" shall mean applying a treatment or cleaning, rinsing, and applying a pretreatment. The pretreatment also functions as a sealant to seal the metal surface, so the term "treating" shall optionally include the step of sealing the metal surface. Further, "treating" optionally can include process steps up through and including painting. For example, treatment steps may also include a step of applying a decorative coating, such as painting. After applying the pretreatment, the pretreatment may be rinsed first or dried-in-place before application of the paint. Each of these steps play a role in a final product's ability to resist corrosion and minimize paint loss. As mentioned above, the treatment composition can be used as a pre-paint treatment.

As used herein, the term "trivalent chromium compound" means compounds, namely salts, of chromium in which the chromium has a valence of plus 3. No hexavalent chromium is present in such compounds. The trivalent chromium compound is a compound with the formula Cr(HₓPO₄)₃, where x is 2 or a compound with the formula Cr(HₓPO₄₎₂, where x is 1.5.

Appropriate concentration ranges of the various components are dependent upon their solubilities. At concentrations too low, there are insufficient amounts of the constituents to cover the metal surface and perform their functions. Above the solubility limits, the solute may begin to come out of the solution. In an embodiment of the invention, the trivalent chromium compound is present in an amount of between: about 10% wt. % to about 5% wt. %; about 10% wt. % to about 2.5% wt. %, about 10% wt. % to about 1% wt. %, or about 10% wt. % to about 0.5% wt. %.. In an embodiment of the invention, the silica is present in an amount of less than 2% wt. %; less than 1.75% wt. %; or less than 1.5% wt. %.

In an embodiment of the invention in which the precursor hexavalent chromium compound is anhydrous chromic acid (CrO₃), the chromic acid is first reduced in the presence of phosphoric acid to create a trivalent chromium compound, chromium dihydrogen phosphate (Cr(H₂PO₄)₃). Hydrogen peroxide is the reducing agent. After the chromium is reduced, silica is added. The following pH range has been found to be preferred given certain other conditions: 1 to 4.

The compositions given above are of the working bath. It is desirable, of course, to transport the product in the form of a concentrate, namely up to a 10 to 100 fold increase in concentration of the above working bath concentrations. The upper limit of such concentrates is the solubility limit of the first constituent to meet or exceed its solubility limit.

The pH of the compositions is preferably, when the composition is used to treat cold rolled steel, between 1 to 4. More preferably, the pH is about 1.75.

Compositions according to the invention may be made by mixing the ingredients in any of a number of sequences. In a non-limiting embodiment where a hexavalent chromium compound is a precursor material, the hexavalent chromium compound is first reduced in the presence of phosphoric acid to create a trivalent chromium compound, chromium dihydrogen phosphate (Cr(H₂PO₄)₃). Hydrogen peroxide is the reducing agent. After the chromium is reduced, silica is added. In another non-limiting embodiment where a hexavalent chromium compound is a precursor material, the hexavalent chromium compound is metered into a solution containing phosphoric acid and hydrogen peroxide until the hexavalent chromium compound is fully reduced. After the chromium is reduced, silica is added.

In one non-limiting embodiment, a concentrate (i.e., master batch) is created by combining the trivalent chromium compound with water. A silica compound can then be added to the solution. The concentrate can then be diluted, preferably with deionized water, to create the desired concentration at the metal treatment site prior to use.

In a non-limiting embodiment, upon completion of the reaction some residual hydrogen peroxide may remain. Conversely, in another non-limiting embodiment, the hydrogen peroxide is fully utilized. Preferably, upon completion of the reaction the hydrogen peroxide concentration is within the following range: from 0 to about 0.85 grams H₂O₂ (35%) per gram of Cr(H₂PO₄)₃.

In a process of the present invention, a metal surface is coated with a pretreatment composition of the present invention. In this coating step, the composition may contact the metal surface by any number of techniques known in the art. One such method is immersion coating in which the metal is immersed in the bath of pretreatment. Other techniques known in the art including spraying, roll coating, or reverse roll coating, as well as manual application (e.g., brushing). The coating step is done for a time sufficient to achieve the desired coating weight on the metal surface, which can be determined empirically. This desired coating weight will depend on a number of factors well-known in the art.

1 milligram per square foot is equal to 10.7639 milligrams per square meter.

In one embodiment, the amount of coating is sufficient to leave from about 0.1 to about 30 milligrams of chromium and phosphate per each square foot of dried metal surface as determined by the weight-strip-weight method. In another embodiment, the amount of coating is sufficient to leave from about 1 to about 10 milligrams of chromium per each square foot of dried metal surface as determined by x-ray fluorescence, and most preferably about 2.5 to about 3.5 milligrams of chromium per each square foot of dried metal surface as determined by x-ray fluorescence. By using a solution with a higher concentration of the included elements, it is possible to leave the desired amount of the dried coating with less residence time.

A process for treating a metal surface to improve corrosion resistance, improve paint adhesion, and/or maintain low electrical contact resistance comprises: (1) cleaning the metal surface to form a cleaned metal surface; (2) rinsing the cleaned metal surface with water to form a rinsed metal surface; and (3) contacting the rinsed metal surface with a composition disclosed herein.

The cleaning step may be carried out in any manner known in the art. The types of cleaners suitable for use in the present invention will vary with a number of factors, including the metal being treated, the desired application, and the amount and type of impurities and soils on the metal surface. As such, the preferred cleaners can be determined empirically based on these factors. In one non-limiting embodiment, an alkaline cleaner is used. An exemplary alkaline cleaning agent which can be used in connection with the present invention is Bulk Kleen^{®} 841MC cleaner, an alkaline liquid cleaner sold by Bulk Chemicals, Incorporated of Reading, Pa. In another non-limiting embodiment, a phosphoric acid cleaner is used. In general, the cleaning step may be accomplished by contacting the metal surface with a bath of an alkaline cleaning solution to form a cleaned metal surface. The alkaline cleaning solution may be an aqueous solution of an alkaline cleaning agent. The cleaning bath cleans the metal surface by removing oil and other contaminants from the metal surface. The cleaning bath is effective to remove the loose impurities and surface soils. Thus, the cleaning bath removes soils and certain impurities from the surfaces of the metal surface. If the metal surface is heavily soiled, a detergent cleaner additive may be included in the cleaning step.

A metal surface which has been contacted by an alkaline cleaning solution is referred to herein as a "cleaned metal surface." It is cleaned in the sense that it has been exposed to a cleaning bath. It may not be completely cleaned, however, in the sense that substantially all of the impurities have been removed such that it is ready to be exposed to a pretreatment composition. In some cases, it may be adequately cleaned, but in other cases, it should first be rinsed with water before being contacted with a pretreatment composition (i.e., substantially all of the impurities are removed by that point).

The rinsing step is well-known in the art, and deionized water is preferably used. The use of deionized water avoids the introduction of any deleterious ions, such as chloride ions, into the system. The rinsing step can be two-fold, with a first rinsing step done using tap water and then rinsing with deionized water.

After step (3) above, contacting the metal surface with the composition, the metal surface may be rinsed with water once again, as is well-known in the art. The rinsed metal surface can then be sealed. Any chemical sealing composition well-known in the industry can be used. When a sealing composition is used, an intervening rinsing step is preferably applied.

After step (3) or any subsequent sealing step, the metal surface may be dried, or rinsed and dried, and then a decorative coating may be applied to it. For example, the metal surface may be painted or lacquered, or first primed and then painted. Such steps, priming and painting, are known in the art as "finishing steps," and any known and suitable finishing steps may be used. Suitable paints include acrylic paints and fluorocarbon paints, among others.

As can be inferred, after step (3) above or any subsequent sealing step, the metal surface can be dried and then a decorative coating (a paint layer) is applied, without an intervening rinsing step between these steps. This alternative process is known as a "dried-in-place" pretreatment. Regardless of whether the pretreatment is "dried-in-place" or there is an intermediate rinsing step, any known method of drying may be employed. The coating may be dried by, for example, using an oven, forced air, etc.

Determining the times of treatments of the metal surfaces with the baths of the various steps is well-known in the art. They need only be long enough to permit a sufficient time for cleaning (in the case of the cleaning step) or reaction (in the case of the pretreatment or sealing steps). They can be very short or as long as thirty minutes and depend on the stage of treatment, the type of application (e.g., immersion, spray), the type of metal surface, and the desired coating weight, among other factors. The immersion time of a substrate into the composition solution will vary with the stage, and generally varies between approximately 1 minute up to about 10 minutes. The times for immersion are typically longer than when spray is used as the method of contact. Rinse times in general can be fairly short, e.g., 30 seconds to one minute. The specific times of treatment may vary over wide ranges and can be readily determined by one of ordinary skill in the art.

The desirable performance characteristics of the present invention can be achieved by the processing steps described above to produce a pretreated metal surface with good paint adhesion and corrosion resistance. These characteristics are obtained on the metal surface without a decorative coating. Accordingly, the treated metal surface can be used as unpainted products and will exhibit corrosion resistance even if there is a delay between the treatment steps and any subsequent painting.

The compositions and processes of the present invention provide the stated benefits without the use of additional components which affect the basic and novel characteristics of the invention. When added to the composition in sufficient amounts, other components may affect the novel characteristics. For example, certain components may make the compositions unstable. Such components may affect the shelf-life of the treatment. Other components may degrade the performance of the compositions and processes of the present invention.

In summary, the present invention provides environmentally friendly compositions and processes for treating metal, while still maintaining excellent paint adhesion and corrosion resistance. More particularly, the present invention avoids the use of hexavalent chromium, and its associated health hazards and disposal problems.

### EXAMPLES

The following examples are included to more clearly demonstrate the overall nature of the invention. Figs. 1-4 illustrate the improved results obtained by employing aqueous compositions of this invention. These examples are exemplary, not restrictive, of the invention.

In the below experiments, a batch of Cr(H₂PO₄)₃ was first synthesized via the combination of the raw materials identified in Table 1 below.

**TABLE 1**

| Raw Material | Mass (g) | Wt. % |
|---|---|---|
| CrO₃ (40%) | 63.5 | 29.1 |
| H₃PO₄ (75%) | 99.5 | 45.6 |
| H₂O₂ (35%) | 55.1 | 25.3 |

A total of 87.1 grams of chromium dihydrogen phosphate (Cr(H₂PO₄)₃) was synthesized. Additional water was added to the solution and the final concentration of the master batch was determined to be 39.2% wt.%. This master batch was further diluted with water to create two separate compositions identified in Table 2 below.

**TABLE 2**

| | Composition 1 | | Composition 2 | |
|---|---|---|---|---|
| Raw Material | Wt. % | Active % | Wt. % | Active % |
| Cr(H₂PO₄)₃ (39.2%) | 22.96 | 9.00 | 15.31 | 6.00 |
| Water | 63.84 | 89.42 | 75.89 | 92.94 |
| Aerodisp W7512S (12%) | 13.20 | 1.58 | 8.80 | 1.06 |

### Preparation of Test Panels - Composition 1

Cold rolled steel panels were treated via the following spray process. First, the panels were cleaned with a 3% v/v solution of Bulk Kleen^{®}841MC for 5 seconds at 74° C. Bulk Kleen^{®}841MC is an alkaline cleaner designed to clean steel, zinc, and aluminum parts. Second, the panels were rinsed at ambient temperature for 30 seconds. Third, the panels were again cleaned with Bulk Kleen^{®}841MC at 3% v/v for 5 seconds at 74° C. Fourth, the panels were rinsed with deionized water at ambient temperature for 30 seconds. Fifth, Composition 1 was applied to the panels using a roll coater. Sixth, the panels were dried using hot air. Seventh, all panels were painted using a high reflectance white, single coat polyester at a dry film thickness of 0.018-0.02 mm.

### Preparation of Test Panels - Composition 2

Cold rolled steel panels were treated via the following spray process. First, the panels were cleaned with a 3% v/v solution of Bulk Kleen^{®}841MC for 5 seconds at 74° C. Second, the panels were rinsed at ambient temperature for 30 seconds. Third, the panels were again cleaned with Bulk Kleen^{®}841MC at 3% v/v for 5 seconds at 74° C. Fourth, the panels were rinsed with deionized water at ambient temperature for 30 seconds. Fifth, Composition 2 was applied to the panels using a roll coater. Sixth, the panels were dried using hot air. Seventh, all panels were painted using a high reflectance white, single coat polyester at a dry film thickness of 0.018-0.02 mm.

### Preparation of Test Panels - Control Formula

Cold rolled steel panels were treated via the following spray process. First, the panels were cleaned with a 3% v/v solution of Bulk Kleen^{®}841MC for 5 seconds at 74° C. Second, the panels were rinsed at ambient temperature for 30 seconds. Third, the panels were again cleaned with Bulk Kleen^{®}841MC at 3% v/v for 5 seconds at 74° C. Fourth, the panels were rinsed with deionized water at ambient temperature for 30 seconds. Fifth, Bulk Bond^{®}780 12% v/v was applied at 74° C in a spray washer for 8 seconds. Bulk Bond^{®}780 is a liquid chemical used in coil coating processes to produce a corrosion-resisting, paint bonding, iron phosphate coating on steel. Afterwards the panels were rinsed with deionized water. Sixth, the panels were dried using hot air. Seventh, the control panels were then sealed with Bulk Bond^{®}NP250 35% v/v using a roll coater. Bulk Bond^{®}NP250 is a liquid chrome/silica product designed to be mill applied as a passivation/pretreatment for multi-metal surfaces. Eighth, all panels were dried and painted using a high reflectance white, single coat polyester at a dry film thickness of 0.018-0.02 mm.

### Preparation of Test Panels - Rausch Formula

Cold rolled steel panels were treated via the following spray process. First, the panels were cleaned with a 3% v/v solution of Bulk Kleen^{®}841MC for 5 seconds at 74° C. Second, the panels were rinsed at ambient temperature for 30 seconds. Third, the panels were again cleaned with Bulk Kleen^{®}841MC at 3% v/v for 5 seconds at 74° C. Fourth, the panels were rinsed with deionized water at ambient temperature for 30 seconds. Fifth, the composition outlined in Example 1 of the Rausch et al. patent was applied to the panels using a roll coater. Sixth, the panels were dried using hot air. Seventh, all panels were painted using a high reflectance white, single coat polyester at a dry film thickness of 0.018-0.02 mm.

All test panels were then exposed to neutral salt spray for a period of 250 or 500 hours per ASTM B117. Photographic comparisons of the results obtained are displayed in Figs. 1-5. As can be seen, Composition 1 and Composition 2 provided comparable protection to the control formula (i.e., Bulk Bond^{®}780) and outperformed the Rausch et al. formula. Specifically, Composition 1 and Composition 2 exhibited similar corrosion and pitting as the control formula, whereas the Rausch et al. formula exhibited increased corrosion and pitting.

Without being bound by any specific theory, it is believed that Composition 1 and Composition 2 outperformed the Rausch et al. formula because of the additional ions other than chromium, phosphate, and silica present in the Rausch et al. formula.

Although illustrated and described above with reference to certain specific embodiments and examples, the present invention is nevertheless not intended to be limited to the details shown. It is expressly intended, for example, that all ranges broadly recited in this document include within their scope all narrower ranges which fall within the broader ranges. It is also expressly intended that the steps of the methods of using the various compositions disclosed above are not restricted to any particular order.

## Claims

1. An aqueous pretreatment composition for treating a metal surface, the composition consisting of:
water;
silica;
a trivalent chromium compound with the formula Cr(H₂PO₄)₃,
and optionally hydrogen peroxide.

2. The aqueous pretreatment composition of claim 1, wherein the pretreatment composition is acidic.

3. The aqueous pretreatment composition of anyone of claims 1-2, wherein the pretreatment composition has a pH of from 1 to 4.

4. The aqueous pretreatment composition of claims 1-3, wherein the aqueous pretreatment composition contains less than 1.75 wt% silica and from 2.5 wt. % to 10 wt. % of the trivalent chromium compound.

5. An aqueous pretreatment composition for treating a metal surface, the composition consisting of:
water;
silica;
a trivalent chromium compound with the formula Cr(H_{1.5}PO₄)₂,
and optionally hydrogen peroxide.

6. The aqueous pretreatment composition of claim 5, wherein the pretreatment composition is acidic.

7. The aqueous pretreatment composition of claims 5-6, wherein the pretreatment composition has a pH from 1 to 4.

8. The aqueous pretreatment composition of claims 5-7, wherein the aqueous pretreatment composition contains less than 1.75 wt% silica and from 2.5 wt. % to 10 wt. % of the trivalent chromium compound.

9. A method for coating a metal surface comprising:
roll coating the metal surface with the composition of claims 1 or 5;
spraying the metal surface for a period of up to 300 seconds in the composition of claims 1 or 5; or
dipping the metal surface for a period of up to 300 seconds with the composition of claims 1 or 5.

10. The method of claim 9 wherein the metal surface is selected from the group consisting of zinc, zinc alloys, aluminum, aluminum alloys, steel, zinc coated steel, and zinc with aluminum alloy.

## Patentansprüche

1. Wässrige Vorbehandlungszusammensetzung zur Behandlung einer Metalloberfläche, wobei die Zusammensetzung besteht aus:
Wasser;
Kieselsäure;
eine dreiwertige Chromverbindung mit der Formel Cr(H₂PO₄)₃, und
optional Wasserstoffperoxid.

2. Wässrige Vorbehandlungszusammensetzung nach Anspruch 1, wobei die Vorbehandlungszusammensetzung sauer ist.

3. Wässrige Vorbehandlungszusammensetzung nach Anspruch 1 oder 2, wobei die Vorbehandlungszusammensetzung einen pH-Wert von 1 bis 4 aufweist.

4. Wässrige Vorbehandlungszusammensetzung nach einem der Ansprüche 1 bis 3, wobei die wässrige Vorbehandlungszusammensetzung weniger als 1,75 Gew.-% Kieselsäure und 2,5 Gew.-% bis 10 Gew.-% der dreiwertigen Chromverbindung enthält.

5. Wässrige Vorbehandlungszusammensetzung zur Behandlung einer Metalloberfläche, wobei die Zusammensetzung besteht aus:
Wasser;
Kieselsäure;
einer dreiwertigen Chromverbindung mit der Formel Cr(H_{1,5}PO₄)₂,
und optional Wasserstoffperoxid.

6. Wässrige Vorbehandlungszusammensetzung nach Anspruch 5, wobei die Vorbehandlungszusammensetzung sauer ist.

7. Wässrige Vorbehandlungszusammensetzung nach Anspruch 5 oder 6, wobei die Vorbehandlungszusammensetzung einen pH-Wert von 1 bis 4 aufweist.

8. Wässrige Vorbehandlungszusammensetzung nach einem der Ansprüche 5 bis 7, wobei die wässrige Vorbehandlungszusammensetzung weniger als 1,75 Gew.-% Kieselsäure und 2,5 Gew.-% bis 10 Gew.-% der dreiwertigen Chromverbindung enthält.

9. Verfahren zum Beschichten einer Metalloberfläche, das folgende Schritte umfasst:
Walzbeschichten der Metalloberfläche mit der Zusammensetzung nach Anspruch 1 oder 5;
Besprühen der Metalloberfläche für eine Dauer von bis zu 300 Sekunden in die Zusammensetzung nach Anspruch 1 oder 5; oder
Eintauchen der Metalloberfläche für eine Dauer von bis zu 300 Sekunden mit der Zusammensetzung nach Anspruch 1 oder 5.

10. Verfahren nach Anspruch 9, wobei die Metalloberfläche aus der Gruppe, bestehend aus Zink, Zinklegierungen, Aluminium, Aluminiumlegierungen, Stahl, verzinktem Stahl und Zink mit Aluminiumlegierung ausgewählt ist.

## Revendications

1. Composition aqueuse de prétraitement pour traiter une surface métallique, la composition consistant en:
eau;
silice;
un composé de chrome trivalent de formule Cr(H₂PO₄)₃,
et éventuellement peroxyde d'hydrogène.

2. Composition aqueuse de prétraitement selon la revendication 1, où la composition de prétraitement est acide.

3. Composition aqueuse de prétraitement selon l'une quelconque des revendications 1 à 2, où la composition de prétraitement a un pH de 1 à 4.

4. Composition aqueuse de prétraitement selon les revendications 1 à 3, où la composition aqueuse de prétraitement contient moins de 1,75 % en poids de silice et de 2,5 % en poids à 10 % en poids du composé de chrome trivalent.

5. Composition aqueuse de prétraitement pour traiter une surface métallique, la composition consistant en:
eau;
silice;
un composé de chrome trivalent de formule Cr(H_{1,5}PO₄)₂,
et éventuellement peroxyde d'hydrogène.

6. Composition aqueuse de prétraitement selon la revendication 5, où la composition de prétraitement est acide.

7. Composition aqueuse de prétraitement selon les revendications 5 et 6, où la composition de prétraitement a un pH de 1 à 4.

8. Composition aqueuse de prétraitement selon les revendications 5 à 7, où la composition aqueuse de prétraitement contient moins de 1,75 % en poids de silice et de 2,5 % en poids à 10 % en poids du composé de chrome trivalent.

9. Procédé de revêtement d'une surface métallique comprenant:
le revêtement au rouleau de la surface métallique avec la composition selon les revendications 1 ou 5;
la pulvérisation de la surface métallique pendant une durée de jusqu'à 300 secondes dans la composition selon les revendications 1 ou 5; ou
l'immersion de la surface métallique pendant une durée de jusqu'à 300 secondes avec la composition selon les revendications 1 ou 5.

10. Procédé selon la revendication 9, où la surface métallique est choisie dans le groupe consistant en le zinc, les alliages de zinc, l'aluminium, les alliages d'aluminium, l'acier, l'acier revêtu de zinc et le zinc avec un alliage d'aluminium.
